

## UNITED STATES PATENT OFFICE

2,335,261

## LUBRICANT

Lloyd L. Davis and Bert H. Lincoln, Ponca City, Okla., assignors, by mesne assignments, to Socony-Vacuum Oil Company, Incorporated, New York, N. Y., a corporation of New York

No Drawing. Application March 21, 1938,  
Serial No. 197,195

3 Claims. (Cl. 252—32)

Our invention relates to lubricants and more particularly to a high quality lubricant containing special soaps.

Modern design in internal combustion engines, and more particularly in Diesel engines, has imposed severe demands on lubricants. In order to properly lubricate modern Diesel engines, the lubricants must be able to maintain a lubricating film at greatly increased loads and at considerably higher temperatures of operation. The severe conditions of use require the lubricants to be more stable than those known to the art. Failure to provide a proper lubricant with modern Diesel engines results in operating difficulties. These demands on lubricants are occasioned, too, by other internal combustion engines though not to the same extent as by Diesel engines.

The failure to supply proper lubricants is evidenced by so-called "sludge" formation, resulting in sticking piston rings and similar troubles. By "sludge" we mean precipitants and matter formed during the operation of the internal combustion engine, which interfere with proper lubrication. Some sludges are hard. Others are adhesive and coherent. Still other sludges are soft and pliable and easily disintegrated.

Probably the most damaging aspect of objectionable sludge results in piston rings sticking. This in turn causes not only increased cylinder wear but frequently scoring of the cylinder walls and sometimes, in severe cases, an actual seizure of the piston by the cylinder walls, due to fusion of metal.

The difficulties which must be overcome cannot be surmounted by changing the character of the hydrocarbon oil, per se. Mineral lubricating oils are peculiarly susceptible to oxidation and sludge formation.

It has been suggested to improve hydrocarbon oils by adding thereto halogenated metallic soaps. Another suggestion to overcome the difficulties mentioned has been to add to hydrocarbon oils small amounts of aromatic substituted stearic acid soaps of calcium. The resulting compositions of matter formed by the hydrocarbon oil and these addition agents have been found to be inadequate. Neither halogenated metallic soaps or calcium soaps of aromatic substituted stearic acid are sufficiently soluble in hydrocarbon oils to give a solution sufficiently stable

under severe operating conditions of use. In order to overcome the solubility difficulty, free fatty acid or free substituted acids have been blended therewith to increase their solubility in hydrocarbon oils. While free acidity helps solubility, it contributes to corrosiveness in the finished lubricant and it has been found that, where bearing compositions containing lead, copper, cadmium and silver are employed, the corrosiveness is such that compositions containing these solubility agents cannot be employed. Lubricants containing these addition agents, furthermore, do not appear to satisfactorily reduce ring sticking difficulty.

Those addition agents of the prior art which have been added to overcome sludge difficulties have not been sufficiently soluble in hydrocarbon oils to give a good stable solution of the required amount of additive. This causes difficulty in the commercial manufacturing and distribution of these lubricants. The defective solubility characteristics of the agents of the prior art is critical and lubricants in which they are used cannot be fortified with a sufficient amount of the addition agents now available to enable the resulting composition to perform its normal duties. When abnormally heavy duties are imposed upon such lubricants, even for short periods of time, sludging occurs, resulting in piston ring sticking and increased cylinder wear.

One object of our invention is to provide addition agents for lubricating oil which will greatly reduce or eliminate ring sticking and which are sufficiently soluble in lubricating oils, including Pennsylvania base oils, solvent treated oils and high viscosity oils, to be effective.

A further object of our invention is to provide a lubricating composition which will substantially reduce or substantially eliminate ring sticking in all internal combustion engines, including airplane engines, automobile engines, and heavy duty internal combustion engines, particularly those of the Diesel type.

Another object of our invention is to provide a lubricant comprising a hydrocarbon oil and an addition agent which is sufficiently soluble in the mineral oils, thereby avoiding the use of acidic solubility agents.

Another object of our invention is to provide

a lubricant containing an addition agent, providing increased film strength, in which the resulting composition is substantially non-corrosive.

Another object of our invention is to provide a lubricant containing an addition agent in which objectionable adhesive sludge formation is minimized.

Another object of our invention is to provide a lubricant containing an addition agent which will convert such sludge as may be formed from mineral oil changes in use into soft, pliable, non-adherent sludge which is unobjectionable.

In general, our invention contemplates the addition of relatively small amounts of special soaps to hydrocarbon lubricating oils.

The particular special soaps used in our invention are made from acids of four types, namely:

a. Acids resulting from the oxidation of petroleum wax or high molecular weight petroleum hydrocarbons.

b. Acids resulting from the oxidation of petroleum wax or high molecular weight petroleum hydrocarbons in which one or more aromatic, aryl, or closed chain radicals have been attached thereto.

c. High molecular weight fatty acids to which are attached one or more aliphatic, alkyl, or open chain radicals.

d. Aromatic or aryl closed chain acids to which are attached one or more long chain aliphatic, alkyl, or open chain radicals.

The inorganic compound to be reacted with the foregoing acids in order to form our special soaps includes the metals, oxides, hydroxides, or salts of:

|           |           |
|-----------|-----------|
| Calcium   | Cadmium   |
| Barium    | Boron     |
| Strontium | Antimony  |
| Magnesium | Chromium  |
| Aluminum  | Cobalt    |
| Tin       | Manganese |
| Zinc      |           |

The above metals are not oxidation catalysts and any other suitable metal of this category can be employed. The metals, lead, iron, copper, and the like, which are oxidation catalysts, are not capable of use in our invention.

Soaps thus formed have many very desirable characteristics, namely:

a. They are very soluble in hydrocarbon oils.  
b. They are sufficiently stable chemically to overcome the tendency to break down in use which results in corrosion.

c. They have very high boiling points which permits them to remain liquid and act as a washing or fluxing material, thus preventing the deposition of sludge-like materials which cause ring sticking.

d. They act to keep sludge-like materials formed in a soft, pliable, non-coherent, and non-adherent condition. (This property results from some mechanism which is not clear to us but is probably related to the molecular size of the materials.)

e. They are relatively non-corrosive at high temperatures.

f. If, under abnormally severe conditions, some slight decomposition takes place, the decomposition products are only weakly acid or alkaline and chemically inactive.

(a) Organic acids of type a, above listed, are normally made by the oxidation of a high boiling

petroleum hydrocarbon, as for example, a paraffin wax or high molecular weight hydrocarbon oils such as petrolatum or bright stock. These hydrocarbons may be oxidized by any of the methods known to the art, by oxygen containing air, gaseous oxygen, or chemical oxidizing agents. The crude oxidation products are separated into acid reacting and non-acid reacting components to obtain the acids suitable for use in compounding the soaps employed in our compositions of matter.

The exact chemical composition of the acids resulting from the oxidation of petroleum hydrocarbons is not known and varies over wide limits, depending upon the particular type of petroleum hydrocarbon subjected to oxidation.

By way of example, a petroleum wax having a melting point of 124°-126° F. was oxidized and acids recovered by precipitating them as insoluble soaps, followed by hydrolysis, to obtain the acids. For convenience, these acids will be termed "wax acids." Calcium soaps, aluminum soaps, zinc soaps, and magnesium soaps of these wax acids were formed and the following compositions of matter concocted:

Calcium-wax acid soaps plus 99.50% SAE 30 mineral oil  
Calcium-wax acid soaps plus 99.00% SAE 40 mineral oil  
Calcium-wax acid soaps plus 98.00% SAE 20 mineral oil  
Aluminum-wax acid soaps plus 99.75% SAE 30 mineral oil  
Aluminum-wax acid soaps plus 99.00% SAE 20 mineral oil  
Aluminum-wax acid soaps plus 98.00% SAE 20 mineral oil  
Zinc-wax acid soaps plus 99.75% SAE 20 mineral oil  
Zinc-wax acid soaps plus 99.00% SAE 40 mineral oil  
Zinc-wax acid soaps plus 98.00% SAE 60 mineral oil  
Magnesium-wax acid soaps plus 99.75% SAE 30 mineral oil  
Magnesium-wax acid soaps plus 99.00% SAE 30 mineral oil  
Magnesium-wax acid soaps plus 98.00% SAE 30 mineral oil  
Magnesium-wax acid soaps plus 96.00% SAE 30 mineral oil

All of the foregoing compositions were of a viscosity only slightly greater than the viscosity of the base mineral oil. All of them were fluid lubricants, that is, none were of the solid or semi-solid grease constituency. Each of the compositions of matter was tested and found satisfactory for accomplishing the objects of our invention.

(b) Petroleum acids (by this is meant acids recovered from the oxidation of hydrocarbon oils) were chlorinated and then subjected to Friedel-Crafts condensations with benzene, naphthalene, and diphenyl to obtain petroleum acids having substituted aromatics, aryl, or closed chain radicals thereon.

The petroleum acid is chlorinated to any desired extent to obtain monochlor, dichlor, trichlor, or polychlor petroleum acids. These chlorinated petroleum acids may be reacted with aromatic compounds as above described.

For example, mono- and trichlor petroleum acids were respectively reacted with approximately one and three molecular equivalents of

the following closed chain radicals to obtain various substituted petroleum acids:

Benzene,  
Xylene,  
Naphthalene,  
Anthracene,  
Benzene with one hydrogen substituted with a radical obtained from chlorinating 124° F.-126° F. melting point wax,  
Naphthalene with one hydrogen substituted with three radicals obtained from chlorinating 124° F.-126° F. melting point wax,  
Cyclohexane,  
Diphenyl,  
Ethyl cyclohexane,  
Octadecal cyclohexane,  
Ethyl diphenyl,  
Di-ethyl diphenyl,  
Octadecal diphenyl,  
Di-octadecyl diphenyl,  
Diphenyl ether,  
Ethyl diphenyl ether,  
Lauryl diphenyl ether,  
Benzophenone,  
Dibutyl benzophenone,  
Triphenyl benzol,  
Ethyl benzoate,  
Lauryl benzoate,  
Furfural,  
Methyl furfural,  
Methyl phenyl pyrrole.

The above substituted petroleum acids were converted into various soaps as follows:

Calcium-monophenyl petroleum acid soap,  
Aluminum-mononaphthyl petroleum acid soap,  
Strontium-anthranyl petroleum acid soap,  
Tin-di-phenyl substituted petroleum acid soap,  
Zinc-octadecyl cyclohexane substituted petroleum acid soap,  
Barium-di-octadecyl diphenyl substituted petroleum acid soap,  
Calcium-benzophenone substituted petroleum acid soap,  
Aluminum-triphenyl benzol substituted petroleum acid soap,  
Calcium-lauryl benzoate substituted petroleum acid soap,  
Aluminum-furfural substituted petroleum acid soap,  
Calcium-methyl phenyl pyrrole substituted petroleum acid soap.

Lubricants were prepared by adding 1.5% of each of the above soaps to 98.5% of a hydrocarbon oil having an SAE viscosity of 30. It was found that metal soaps of aromatic substituted petroleum acids accomplish the objects of our invention and are suitable as addition agents to hydrocarbon oils to minimize piston ring sticking.

(c) The organic acids may be easily prepared by substituting one or more large petroleum hydrocarbon molecules on the various fatty acids and the resulting product converted into the various soaps.

Petroleum is a mixture of hydrocarbons of varying molecular weight; but by selecting a comparatively close boiling range material, it is possible to minimize the number of different hydrocarbon molecules in the cut. To accomplish the objectives of this invention, it is not necessary to employ a pure petroleum hydrocarbon; nor is it necessary to have a close fractionated cut.

Whatever fraction of crude petroleum that is selected will prove satisfactory, but it is desirable to select a fraction having a boiling point above about 150° F. The various fatty acids may be used; but if a low molecular weight fatty acid is used, then at least one high molecular weight petroleum hydrocarbon should be attached to it, or two or more of the lower molecular weight petroleum hydrocarbons should be attached to it.

10 For example, with acetic acid a petroleum hydrocarbon of the wax boiling range should be employed or two hydrocarbons of the kerosene boiling range. With stearic acid one or more of the high or low boiling range, or high or low molecular weight, petroleum hydrocarbons may be employed.

15 Some of the normal fatty acids which may be employed herein are acetic, propionic, butyric, capric, lauric, palmitic, stearic, caranaubic, melissic, oleic, linoleic, ricinoleic, and the like.

To the foregoing fatty acids may be attached one or more aliphatic hydrocarbons of from six to fifty carbon atoms. The cheapest source of these hydrocarbons is petroleum oil; therefore hydrocarbons or fractions of comparatively narrow boiling range from the gasoline, kerosene, gas oil, lubricating oil or wax boiling range may be employed. Obviously hydrocarbons similar to those from petroleum may be employed regardless of source, or pure synthetic hydrocarbons may be employed. By "aliphatic hydrocarbons" we include the hydrocarbons obtainable from petroleum oil regardless of the source.

This invention is not limited to the method of combining the fatty acids and the aliphatic hydrocarbons since any of the well known methods of addition or substitution may be employed.

25 Stearic acid with one, two, and four substituents from a wax having a melting point of 124°-126° F. was formed and converted into various soaps. Oleic acid, with as many as six substituents from a hydrocarbon boiling within the gasoline boiling range were formed and converted into various soaps.

30 A number of aliphatic substituted fatty acids were formed, as for example:

Calcium-stearic-monowax hydrocarbon soap,  
Calcium-stearic-diwax hydrocarbon soap,  
Calcium-stearic-triwax hydrocarbon soap,  
Calcium-stearic-tetrawax hydrocarbon soap,  
Aluminum-oleic-monokerosene hydrocarbon soap,  
Aluminum-oleic-dikerosene hydrocarbon soap,  
Aluminum-oleic-trikerosene hydrocarbon soap,  
Aluminum-oleic-tetrakerosene hydrocarbon soap,  
Zinc-caranaubic-monowax hydrocarbon soap,  
Zinc-caranaubic-diwax hydrocarbon soap,  
Zinc-caranaubic-triwax hydrocarbon soap,  
Zinc-caranaubic-tetrawax hydrocarbon soap,  
Tin-caranaubic-monogasoline hydrocarbon soap,  
Tin-caranaubic-digasoline hydrocarbon soap,  
Tin-caranaubic-trigasoline hydrocarbon soap,  
Tin-caranaubic-tetragasoline hydrocarbon soap.

65 Compositions of matter were compounded containing 98.5% of an SAE 20 hydrocarbon oil and 1.5% of metal soaps of aliphatic substituted fatty acids and these were found to accomplish the objects of our invention.

70 (d) The organic acids of class d above, are prepared from aromatic or closed chain acids with one or more high molecular weight substituents such as wax hydrocarbon substituents on an aromatic nucleus. Some of the ring or closed chain acids which are satisfactory for the

introduction of a high molecular weight substituent are:

Benzoic,  
Methyl benzoic,  
Salicylic,  
Phenyl salicylic,  
Phenyl acetic,  
Phenyl propionic,  
Cinnamic,  
Phthalic,  
Terephthalic,  
Isophthalic,  
Phenyl butyric,  
Anthranilic,  
Hypuric,  
Uric phenanthrene carboxylic,  
Phenanthrene dicarboxylic,  
Phenyl glycollic,  
Hydroxytropic acridimic,  
Azulmic,  
Pyrazole carboxylic acids,  
Pyrazole dicarboxylic acid,  
Furan carboxylic acids,  
Furan dicarboxylic acids,  
Furoxan carboxylic acids,  
Pyrrole carboxylic acids.

One or more aliphatic or open chain radicals may be attached to these ring acids. The aliphatic radical may contain from four to fifty carbon atoms. Any of the petroleum hydrocarbons having the requisite number of carbon atoms may be employed.

The aliphatic hydrocarbon radicals may be introduced into the ring compound by any of the well known methods such as by the Friedel-Crafts reaction or one of its modifications. If the Friedel-Crafts reaction is employed to introduce the open chain radical into the closed acid chain, then either one, two, three or more halogens may be introduced into the aliphatic radical, depending on whether the mono-, di-, or tri-substitution product is desired.

A number of aliphatic substituted ring acids were formed and converted into soaps as follows:

Calcium-benzoic-monowax hydrocarbon soap  
Calcium-benzoic-diwax hydrocarbon soap  
Calcium-benzoic-triwax hydrocarbon soap  
Aluminum-phenylacetic-monokerosene hydrocarbon soap  
Aluminum-phenylacetic-dikerosene hydrocarbon soap  
Aluminum-phenylacetic-trikerosene hydrocarbon soap  
Zinc-phthalic acid-monogasoline hydrocarbon soap  
Zinc-phthalic acid-digasoline hydrocarbon soap  
Zinc-phthalic acid-trigasoline hydrocarbon soap  
Zinc-phthalic acid-monowax hydrocarbon soap  
Calcium-phthalic acid-monowax hydrocarbon soap  
Calcium-phthalic acid-monokerosene hydrocarbon soap  
Aluminum-phthalic acid-monowax hydrocarbon soap  
Aluminum-phthalic acid-monokerosene hydrocarbon soap

Compositions of matter were formed in which 70  
1.5 percent of the aliphatic substituted ring acid

metal soaps were added to 98.5 percent of an SAE 30 mineral oil and were found to accomplish the objects of our invention.

It is to be understood that the examples above given are by way of illustration only and not by way of limitation and that any soaps of the following group are of use in our invention:

Metal soaps of petroleum acids  
Metal soaps of substituted petroleum acids  
10 Metal soaps of aliphatic substituted fatty acids  
Metal soaps of aliphatic substituted aromatic acids.

It will be observed that, broadly stated, our invention comprises the addition to a hydrocarbon oil of small amounts of metal soaps of acids selected from the following group:

- a. Petroleum acids (that is, acids obtained by the oxidation of petroleum hydrocarbons)
- 20 b. Substituted petroleum acids
- c. Aliphatic substituted organic acids
  1. Fatty acids
  2. Aromatic acids.

25 The amount of soaps to be used varies over wide limits. The smallest amount which might be used practically is about one fourth of one percent. The highest concentration of the addition agent would not be more than fifteen percent. A 30 preferential range for practice would be between one half of one percent and five percent. For engines of the Diesel type, a concentration of three fourths of one percent to two percent of the addition agents has been found satisfactory. All 35 of the soaps of the various acids are not equal in effectiveness and it will be found, therefore, that the wide percentage range of one fourth of one percent to fifteen percent will be sufficiently broad to provide for variations in effectiveness.

40 All of the addition agents, however, do have the properties pointed out, namely of preventing piston ring sticking difficulties by causing such sludge as is formed to be of the soft, non-adherent character.

45 It will be understood that certain features and sub-combinations are of utility and may be employed without reference to other features and sub-combinations. This is contemplated by and is within the scope of our claims. It is further 50 obvious that various changes may be made in details within the scope of our claims without departing from the spirit of our invention. It is, therefore, to be understood that our invention is not to be limited to the specific details shown 55 and described.

Having thus described our invention, what we claim is:

1. A lubricant comprising in combination a hydrocarbon oil and from one fourth of one percent to fifteen percent by weight of a metal soap of an aliphatic substituted fatty acid.
2. A lubricant comprising in combination a hydrocarbon oil and from one half of one percent to five percent by weight of a metal soap of an aliphatic substituted organic acid.
3. A lubricant comprising in combination a hydrocarbon oil and from one half of one percent to five percent by weight of a metal soap of an aliphatic substituted ring acid.

LLOYD L. DAVIS.  
BERT H. LINCOLN